

# UNITED STATES PATENT OFFICE.

PHILIP M. MCKENNA, OF CONGRESS HEIGHTS, DISTRICT OF COLUMBIA.

## ALLOY STEEL.

1,389,680.

Specification of Letters Patent.

Patented Sept. 6, 1921.

No Drawing.

Application filed April 2, 1921. Serial No. 458,032.

*To all whom it may concern:*

Be it known that I, PHILIP M. MCKENNA, a citizen of the United States, residing at Congress Heights, in the District of Columbia, have invented certain new and useful Improvements in Alloy Steel; and I do hereby declare the following to be a full, clear, and exact description of the same.

This invention relates to the steel industry and more especially to that branch of the industry having to do with alloy steels, the objects of the invention being to produce an alloy steel which is tough and strong and possesses an evenness of grain which makes it valuable for use in machine parts subject to shock and strain or in other situations where a uniformly strong metal is desired, as, for example, in springs, gun barrels, saws, etc.

20 The invention consists in an alloy steel which besides iron contains carbon, chromium and tantalum as the characteristic imparting elements, although there may be present, incidentally, impurities in negligible quantity, such as sulfur, phosphorus, silicon, manganese, columbium, vanadium, etc.

The alloy of the present invention contains not less than .20 per cent. of carbon, preferably carbon .20 to .50 per cent., chromium .70 to 1.60 per cent., and tantalum 1 to 3 per cent. with the remainder iron, save for the impurities present in the ingredients and which it is difficult to entirely eliminate.

The alloy may be readily produced in electric or in other suitable steel melting furnaces. If it is produced in the open-hearth furnace the ferro-tantalum should be added

to the ladle, and not to the furnace. The ingredients, with the exception of the tantalum, (and a small amount of iron which is added in the ferro-tantalum) are first melted in the furnace. If an electric furnace is used the ferro-tantalum is added to the molten bath, quick tests are taken until the percentage of carbon is adjusted, and the metal is poured. If an open-hearth furnace is used the molten metal is run into a ladle, after the quick tests show the ingredients to exist in the right proportions with the exception of the ferro-tantalum. Then the ferro-tantalum is added to the ladle.

The ferro-tantalum may be produced by reducing tantalite or columbite with iron oxid, in an electric furnace, or by aluminothermic reaction. This will result in a ferro-alloy containing about 30 per cent. tantalum. It is very essential to use only tantalite or columbite ore which is free from deleterious impurities such as tin, antimony, copper, sulfur, arsenic and phosphorus which otherwise go into the alloy and cause the metal to be subject to breakage, and lose its valuable physical properties. The ferro-alloy is added to the molten bath in pieces about the size of peas, in order that the metal may readily absorb the ferro-tantalum.

The metal produced can be worked up into shapes by forging and can be hardened and tempered without cracking.

What I claim is:

An alloy containing, besides iron, not less than .20 per cent. carbon, .70 to 1.60 per cent. chromium, and 1 to 3 per cent. of tantalum.

PHILIP M. MCKENNA.

70